# EUROPEAN PATENT SPECIFICATION

(11) **EP 0 406 001 B1**
(45) Date of publication and mention of the grant of the patent: **08.05.1996**
(21) Application number: 90307130.6
(22) Date of filing: 29.06.1990
(51) Int. Cl.: G03G 5/06, G03G 5/05

(54) **Matrix plate for electrophotographic platemaking and printing plate**
Matrixplatte für die elektrophotographische Herstellung von Druckplatten und Druckplatte
Plaque matrice pour la fabrication électrophotographique de plaques d'impression et plaque d'impression

(30) Priority: 29.06.1989 JP 165231/89; 25.06.1990 JP 166349/90
(43) Date of publication of application: 02.01.1991
(73) Proprietor: NIPPON SHOKUBAI CO., LTD., Osaka-shi (JP)
(72) Inventor: Kaieda, Osamu, Tsukuba-shi, Ibaragi-ken (JP); Masuda, Kiyoshi, Ushiku-shi, Ibaraki-ken (JP); Ito, Hideki, Tsukuba-shi, Ibaraki-ken (JP); Yodoshi, Takashi, Tsukuba-shi, Ibaraki-ken (JP)
(74) Representative: Rees, David Christopher

(56) References cited:
- GB-A- 2 059 348
- US-A- 4 461 818
- PATENT ABSTRACTS OF JAPAN , Vol. 13, no. 236 (C-602)(3584) 30 May 1989 ( NIPPON SHOKUBAI KAGAKU KOGYO CO., LTD. ) 17 February 1989 & JP-A-145 474

## Description

This invention relates to a matrix plate for electrophotographic platemaking and a printing plate obtained by exposing to radiation and developing the matrix plate. More particularly, it relates to a plate-making matrix plate sensitive to a semiconductor laser and capable of directly making a plate by the electrophotographic process and a printing plate obtained by exposing to radiation and developing the matrix plate.

The technological advances in computer image processing and mass storage communication have recently encouraged proposal as a new system of the so-called phototelegraphic printing to be effected by processing a given image with a computer thereby obtaining image information in the form of a digital signal, electrically transmitting the image information with a telephone circuit or a communications satellite, subjecting the image information reaching the receiver to the operation of a scanner device on the receiver's side, and irradiating this image information with a laser in the scanning manner.

The conventional matrix plate for platemaking has relied predominantly on the method using photosensitive resin (PS plate method). In the case of the PS plate method, since the platemaking is accomplished by causing the received information to be written in a silver salt film as a provisional step, pressing the film fast against a matrix plate, and exposing the film to radiation, this method has a disadvantage that the plate-making operation necessitates a voluminous apparatus and consumes much time. Further, most photosensitive materials for the PS plate method make use of a photochemical reaction and, therefore, require ample exposure to radiation and generally are deficient in sensitivity. Thus, the photosensitive materials of the PS plate method have a disadvantage that they are incapable of producing fully satisfactory image information by the exposure to a low-output inexpensive semiconductor laser.

For the solution of the problems of the PS plate method described above, a method which uses a silver halide photosensitive material for photo-making matrix plate and a method which utilizes the electrophotographic process have been proposed and partly put to practical use. Though the former method enjoys highly satisfactory sensitivity, it suffers from a disadvantage that the plate is deficient in resistance to the impact of printing and is unduly expensive. In contrast, the latter method allows direct platemaking, enjoys relatively high senistivity and inexpensiveness, and promises successful production of a printing plate highly resistant to the impact of printing. Thus, it has been the subject of active study in recent years.

In the matrix plate for electrophotographic platemaking, zinc oxide and organic compounds have been used as photoelectroconductive substances. The plate-making matrix plate using zinc oxide generally suffers from disadvantages such as (A) the fact that the produced printing plate tends to be defiled because the non-image part thereof is deficient in hydrophilicity, (B) the fact that the produced printing plate is deficient in resistance to the impact of printing because it suffers the photosensitive layer to peel off under the mechanical pressure exerted thereon during the course of printing or owing to the permeation therein of the dampening water, and (C) the fact that the produced printing plate, in spite of sensitization with pigment performed in advance thereon for impartation of sensitivity to the region of visible light, exhibits no fully satisfactory sensitivity in the region of long wavelength exceeding 600 nm and allows no easy effective exposure with a semiconductor laser.

In the case of the plate-making matric plate using a photoelectroconductive organic compound, the platemaking is accomplished by dispersing the photoelectroconductive organic compound in a binder resin formed mainly of an alkali-soluble resin thereby preparing a photosensitive material, applying the photosensitive material to an abraded surface of a substrate such as of aluminum sheet thereby superposing a photosensitive layer on the substrate, forming a toner image by the electrophotographic technique on the photosensitive layer, and dissolving and removing the non-image part with an alkali extractant.

Numerous electrophotographic plate-making matric plates have been proposed which are provided with a photosensitive layer having a varying photoelectroconductive organic compound dispersed in an alkali-soluble resin. For example, JP-A-54-134,632(1979), JP-A-55-105,254(1980), and JP-A-55-153,948(1980) disclose such matrix plates using phenol resin as the alkali-soluble resin. When a phenol resin is used as a binder resin for such a photoelectroconductive organic compound, however, the produced film has a disadvantage that it is brittle and, therefore, deficient in resistance to the impact of printing.

JP-A-58-76,843(1983), JP-A-59-147,355(1984), JP-A-60-17,752(1985), JP-A-60-243,670(1985), JP-A-62-198,864(1987), and JP-A-64-23,260(1989) disclose matric plates using a styrene-maleic acid copolymer as the alkali-soluble resin. When a styrene-maleic acid copolymer is used as a binder resin for a photoelectroconductive organic compound, however, there arises a disadvantage that the produced film is so hard that the printing plate tends to sustain cracks when it is bent. Acrylic resins have been employed in many cases. JP-A-54-89,801(1979) discloses a matric plate using an aqueous acrylic resin as a binder resin and an ε type crystalline copper phthalocyanine as a photoelectroconductive organic compound. These matrix plates are capable of forming an image by the electrophotographic process. They, however, suffer from a disadvantage that they are not easily etched with an aqueous alkali solution and are incapable of effective exposure to a radiation in the near infrared region such as a semiconductor laser.

JP-A-56-146,145(1981) discloses a method which uses as a binder resin such an acrylic resin as an acrylic acid/methyl methacrylate/butyl acrylate copolymer, for example, and as photoelectroconductive organic compounds a condensed polycyclic quinone type pigment and an oxadiazole derivative. Though the matric plate obtained by this method allows an etching treatment to be effected easily with an aqueous alkali solution, it has a disadvantage that it possesses no fully satisfactory electrophotographic properties and shows poor stability to withstand storage for an extended period. It also has a disadvantage that it is incapable of effective exposure to radiation in the near infrared region such as a semiconductor laser. It has a problem of inferior resistance to the impact of printing because it is incapable of effective exposure to radiation in the near infrared region such as a semiconductor laser or, if it is adapted somehow or other to attain the exposure, it exhibits no fully satisfactory behavior as in the electrophotographic properties.

JP-A-64-145474 discloses the use of a fluorine-containing phthalocynaine compound as a photo electroconductive material in optical information recording media.

An object of this invention, therefore, is to provide a novel matrix plate for electrophotographic platemaking and a printing plate produced by exposing to radiation and developing this matrix plate.

Another object of this invention is to provide an electrophotographic plate-making quality matrix plate resorting to an improved method using a photoelectroconductive organic compound and a lithographic printing plate.

A further object of this inventionis to provide an electrophotographic plate-making quality matrix plate excelling in electrophotographic properties and alkali-extractability and a lithographic printing plate excelling in printing properties.

Still another object of this invention is to provide an electrophotographic plate-making quality matrix plate capable of producing a printing plate excelling in stability to withstand storage for an extended period and resistance to the impact of printing.

Yet another object of this invention is to provide an electrophotographic plate-making quality matrix plate which is furnished with a photosensitive layer excelling in lightfastness and weatherability owing to the use of a binder resin possession highly satisfactory fast adhesiveness to a substrate and satisfactory mechanical strength.

A further object of this invention is to provide an electrophotographic plate-making quality matrix plate exhibiting high sensitivity even in the region of near infrared wavelength and allowing effective exposure to a semiconductor laser.

The objects described above are accomplished by an electrophotographic matrix plate comprising an electroconductive substrate having a photosensitive layer comprising an alkali-soluble binder resin and a photoconductive fluorinated zinc phthalocyanine compound, which matrix plate is characterized in that the photoconductive compound is an octafluoro zinc phthalocynaine represented by the general formula I: wherein R is a -SZ group (where Z is a phenyl group, a phenyl substituted with an alkyl group of 1 to 5 carbon atoms, or a naphthyl group), and the binder resin is a copolymer obtainable by polymerizing a monomer mixture comprising (a) at least one compound selected from the group consisting of hydroxyalkyl acrylates and hydroxyalkyl methacrylates, (b) at least one copolymerizable unsaturated carboxylic acid, (c) at least one styrene compound, and (d) at least one compound selected from among acrylic esters other than the hydroxyalkyl acrylates of (a), and optionally (e) at least one methacrylic ester other than the hydroxyalkyl methacrylates of (a).

The objects described above are also accomplished by a lithographic printing plate which is produced by forming a toner image by the electrophotographic process on the electrophotographic plate-making matrix plate described above, fixing the toner image, and removing the non-image part with an alkaline etching liquid.

Since the electrophotographic process on the electrophotographic plate-making matrix plate of the present invention is constructed as described above, it produces the following effects.
(1) It is excellent in electrophotographic properties and capable of effecting electrophotographic platemaking with high efficiency.
(2) It excels in alkali-extractability and allows required etching to be carried out effectively during the course of a plate-making process.
(3) It allows the photosensitive layer thereof to be produced with a low phthalocyanine content in a small wall thickness without adversely affecting the highly desirable states of electrophotographic properties (chargeability and sensitivity).
(4) Since it exhibits highly satisfactory sensitivity even in the region of long wavelength, it can be given effective exposure with not only an ordinary light source such as a tungsten lamp but also a low-output laser. As the result, it allowed direct platemaking to be attained with a varying light source.
(5) The binder resin has high affinity for zinc phthalocyanine and exhibits highly satisfactory dispersibility therein.
(6) The printing plate obtained by the electrophotographic plate-making technique excels in printing properties and allows production of clear prints even after 100,000 cycles of repeated use. It also excels in stability to withstand storage for an extended period.

The electrophotographic plate-making quality matrix plate according with the present invention is provided on an electroconductive substrate with a photosensitive layer. This photosensitive layer is formed of an alkali-soluble binder regin containing a photoelectroconductive organic compound.

The photoelectroconductive organic compound to be used in the present invention is a zinc phthalocyanine represented by the aforementioned general formula I. This size phthalocyanine excels in electrophotographic properties even when it is contained in the alkali-soluble binder regin and refrains from interfering with alkali-extractability.

As concrete examples of the zinc phthalocyanines represented by the aforementioned general formula (I), the following compounds may be cited. Invariably in these compounds, a total of eight fluorine atoms are inorporated one each at the 1, 4, 5, 8, 9, 12, 13 and 16 positions of a phthalocyanine nucleus represented by the following formula (II). The formulas enclosed with brackets [ ] are abbreviations.

Octafluoro-octakis(phenylthio) zinc phthalocyanine [F₈(PhS)₈ZnPc],
Octafluro-octakis(o-tolylthio) zinc phthalocyanine [F₈(o-MePhS)₈ZnPc],
Octafluro-octakis(m-tolylthio) zinc phthalocyanine [F₈(m-MePhS)₈ZnPc],
Octafluro-octakis(m-tolylthio) zinc phthalocyanine [F₈(p-MePhS)₈ZnPc],
Octafluoro-octakis (2,4-xylylthio) zinc phthalocyanine [F₈(2,4-MePhS)₈ZnPc],
Octacluoro-octakis(2,3-xylylthio) zinc phthalocyanine [F₈(2,3-MePhS)₈ZnPc],
Octafluoro-octakis(o-ethylphenylthio) zinc phthalocyanine [F₈(o-EtPhS)₈ZnPc],
Octafluoro-octakis(p-ethylphenylthio) zinc phthalocyanine [F₈(p-EtPhS)₈ZnPc],
Octafluoro-octakis(o-isopropylphenylthio) zinc phthalocyanine [F₈(o-IPrPhS)₈ZnPc],
Octafluoro-octakis(o-butylphenylthio) zinc phthalocyanine [F8(o-BUPhS)₈ZnPc],
Octafluoro-octakis(m-butylphenylthio) zinc phthalocyanine [F₈(m-BuPhS)₈ZnPc],
Octafluoro-octakis(p-butylphenylthio) zinc phthalocyanine [F₈(p-BuPhS)₈ZnPc],
Octafluoro-octakis(p-tertiary butylphenylthio) zinc phthalocyanine [F₈(p-t-BuPhS)₈ZnPc], and
Octafluoro-octakis(naphthylthio) zinc phthalocyanine [F₈(NPhS)₈ZnPc]

The zinc phthalocyanine represented by the general formula I can be produced as follows from 3,4,5,6-tetrafluorophthalonitrile, for example, as a starting material. In an organic solvent such as methanol or acetonitrile, 3,4,5,6-tetrafluorophthalonitrile is caused to react with RSH, RSNa, or RSK, wherein R is a phenyl group or a naphthyl group, for example, in the presence of a condensing agent such as an alkaline substance (KF, for example) to synthesize 3,4,5,6-tetrafluorophthalonitrile having functional groups substituted in advance on each for the fluorine atoms at the 4 and 5 positions thereof. Then, by causing the resultant phthalonitrile now incorporating therein the substituents and zinc powder or a zinc halide to be fused by heating or to be heated in an organic solvent, the zinc phthalocyanine mentioned above is obtained.

The binder resin to be used in the present invention is a copolymer obtained by polymerizing a monomer mixture comprising (a) at least one compound selected from the group consisting of hydroxyalkyl acrylates and hydroxyalkyl methacrylates, (b) at least one copolymerizable unsaturated carboxylic acid, (c) at least one styrene compound, and (d) at least one compound selected from among acrylic esters other than hydroxyalkyl acrylates of (a).

The monomer of (a) is at least one compound selected from among hydroxyalkyl acrylates and hydroxyalkyl methacrylates having hydroxyalkyl groups of 2 to 10, preferably 2 to 6, carbon atoms (hereinafter acrylic acid and methacrylic acid will be collectively referred to as "(meth)acrylic acid"). Specifically, the hydroxyalkyl (meth)acrylates which are usable herein include 2-hydroxyethyl (meth)acrylates, 2-hydroxypropyl (meth)acrylates, 3-hydroxypropyl (meth)acrylates, 2-hydroxybutyl (meth)acrylates, glycerol mono(meth)acrylates, and trimethylol propane (meth)acrylates, for example. The use of the monomer (a) results in improving the electrophotographic properties and the durability as a printing plate. It also contributes to producing a uniform and pretty coating. This favorable effect may be logically explained by a postulate that the introduction of the hydroxy group in the binder regin enhances the fast adhesiveness of the binder regin to the electroconductive substrate and, at the same time, heightens the affinity of the binder regin for the phthalocyanine of the present invention to the extent of improving the dispersibility. It is also effective in heightening the alkali etching property and allowing a decrease in the proportion of the copolymerizable unsaturated carboxylic acid which is liable to impair electrophotographic properties when used in a high ratio.

The ratio of the monomer of (a) to be used is in the range of 0.5 to 40% by weight, preferably 2 to 25% by weight, based on the total amount of the mixed monomer. If this ratio is less than 0.5% by weight or not less than 40% by weight, there arises a disadvantage that the electrophotographic properties and the durability of printing plate are degraded.

The monomer of (b) is at least one copolymerizable unsaturated carboxylic acid. The copolymerizable unsaturated carboxylic acids which are usable herein include such unsaturated monomers as monocarboxylic acids represented by (meth)acrylic acids; dicarboxylic acids represented by maleic acid, itaconic acid, and citraconic acid and dicarboxylic monoesters represented by monoisopropyl maleate which have at least one carboxyl group in the molecular unit thereof. Among other unsaturated monomers mentioned above, (meth)acrylic acids and/or itaconic acid prove to be advantageously useful. The ratio of the monomer of (b) to be used herein is in the range of 10 to 40% by weight, preferably 15 to 30% by weight, based on the total amount of the monomer mixture. If this ratio is less than 10% by weight, there follows a disadvantage that the alkali-solubility of the produced copolymer is unduly low and the etching speed is proportionally low. Conversely, if this ratio exceeds 40% by weight, the photosensitive layer is too deficient in chargeability to be used effectively. For the purpose of acquiring a highly desirable etching property, the copolymer to be used as the binder regin of the present invention may incorporate therein a carboxylic acid so much as to adjust the acid value thereof in the range of 50 to 300 mg-KOH/g. By using the copolymerizable carboxylic acid in the specific range mentioned above, the etching property can be improved without impairing the electrophotographic properties.

The monomer of (c) is a styrene compound. The styrene compounds which are effectively usable herein include styrene and alkyl styrenes such as methyl styrene, ethyl styrene, and isopropyl styrene, for example. Among other styrene compounds mentioned above, styrene proves to be particularly preferable. The ratio of the monomer of (c) to be used is in the range of 10 to 70% by weight, preferably 25 to 55% by weight, based on the total amount of the monomer mixture. If this ratio is less than 10% by weight, there ensues a disadvantage that the strength, the affinity (dispersibility) for phthalocyanine, and the chargeability are unduly low. Conversely, if this ratio exceeds 70% by weight, there ensues a disadvantage that the aforementioned effects due to the use of the monomers of (a) and (b) are no longer manifested because the ratios of the monomers of (a) and (b) are proportionately decrease.

The monomer of (d) is at least one compound selected from among the acrylic esters other than the hydroxyalkyl acrylates usable for the monomer of (a). The acrylic esters which are usable effectively herein include alkyl acrylates having alkyl groups of 1 to 12, preferably 2 to 8, carbon atoms and cycloalkyl acrylates having cycloalkyl groups of 5 to 7 carbon atoms. As typical examples of alkyl acrylates and cycloalkyl acrylates are methyl acrylate, ethyl acrylate, isopropyl acrylate, n-propyl acrylate, 2-ethylhexyl acrylate, lauryl acrylate, cyclohexyl acrylate, and cycloheptyl acrylate. The ratio of an alkyl acrylate or cycloalkyl acrylate to be used is in the range of 5 to 50% by weight, preferably 10 to 40% by weight, based on the total amount of the monomer mixture. So long as this ratio is in the range mentioned above, the added alkyl acrylate or cycloalkyl acrylate enhances the oleophilicity and the produced copolymer enjoys increased binding force and improved flexibility. If this ratio exceeds 50% by weight, there ensues a disadvantage that the aforementioned effects brought about by the use of the monomers of (a), (b) and (c) are no longer manifested because the ratios of the monomers of (a), (b), and (c) are proportionately decreased. The monomer of (e) which is used as occasion demands in the present invention is at least one compound selected from methacrylic esters other than the aforementioned hydroxyalkyl methacrylates. Specifically, the methacrylic esters which are usable herein are alkyl methacrylates having alkyl groups of 1 to 12, preferably 2 to 8, carbon atoms and cycloalkyl methacrylates having cycloalkyl groups of 5 to 7 carbon atoms.

As typical examples of the alkyl methacrylates and cycloalkyl methacrylates, there may be cited methyl methacrylate, ethyl methacrylate, n-propyl methacrylate, isopropyl methacrylate, n-butyl methacrylate, isobutyl methacrylate, sec-butyl methacrylate, t-butyl methacrylate, 2-ethylhexyl methacrylate, cyclohexyl methacrylate, and cycloheptyl methacrylate. The ratio of an alkyl methacrylate or cycloalkyl methacrylate to be used is in the range of 0 to 40% by weight, preferably not more than 15% by weight. So long as this ratio is in the range mentioned above, the added methacrylate goes to enhancing the durability. If this ratio exceeds 40% by weight, however, there ensues a disadvantage that the dispersibility of phthalocyanine is impaired.

Of the various monomer mixtures indicated above, typical monomer mixtures (p-1) to (p-10) indicated below have the compositions and monomer ratios as indicated.
(p-1) 2-Hydroxypropyl acrylate/acrylic acid/styrene/butyl acrylate (5/20/35/40) (by weight; which invariably applies hereinafter)
(p-2) 2-Hydroxyethyl methacrylate/methacrylic acid/styrene/butyl acrylate (2/23/40/35),
(p-3) 2-Hydroxybutyl methacrylate /acrylic acid/styrene, isopropyl acrylate (15/25/45/15),
(p-4) 3-Hydroxypropyl methacrylate/acrylic acid/styrene/methyl acrylate/ethyl methacrylate (5/20/35/25/15),
(p-5) 3-Hydroxybutyl acrylate/methacrylic acid/styrene/isobutyl acrylate/isopropyl methacrylate (20/30/25/20/5),
(p-6) 2-Hydroxyethyl methacrylate/methacrylic acid/styrene/propyl acrylate/ethyl methacrylate (5/25/40/25/5),
(p-7) 2-Hydroxybutyl methacrylate/itaconic acid/styrene/butyl acrylate/methyl methacrylate (10/15/35/30/10), and
(p-8) 3-Hydroxybutyl acrylate/acrylic acid/styrene/ethyl acrylate/butyl acrylate/butyl methacrylate (5/20/25/4/10).

No particular method is specified for the polymerization of the aforementioned monomer mixture. For example, the monomer mixture can be polymerized by any of the conventional polymerization methods such as the bulk polymerization method, solution polymerization method, and suspension polymerization method in the presence of a radical polymerization initiator such as a peroxide, a hydroperoxide, or azobisisobutylonitrile at a temperature in the range of 50° to 100°C, preferably 70° to 90°C. As regards the manner of addition of the monomer mixture, the method of collective addition, split addition, continuous addition, or a suitable combination thereof may be used.

The number average molecular weight of the copolymer obtained by polymerizing the monomer mixture is in the range of 1,000 to 50,000, preferably 3,000 to 30,000.

The copolymer which is obtained by polymerizing the monomer mixture and which has a number average molecular weight in the range mentioned above is soluble in an alkaline substance. The photosensitive layer which is obtained by applying this copolymer in combination with the aforementioned photoelectroconductive phthlocyanine compound exhibits highly satisfactory alkali-solubility and excels in etching property.

The electrophotographic plate-making quality matrix plate of the present invention is a product obtained by preparing a coating liquid consisting of the aforementioned photoelectroconductive phthalocyanine compound and the aforementioned copolymer as a binder resin and applying the coating liquid to an electroconductive substrate thereby forming a photosensitive layer thereon.

The method for the preparation of the coating liquid is not particularly limited. The preparation may be attained by dissolving or dispersing the binder resin (or the photoelectroconductive phthalocyanine compound) in a suitable solvent and then dissolving or dispersing the photoelectroconductive compound (or the binder regin) in the resultant solution or by dissolving or dispersing the binder regin and the photoelectroconductive phthalocyanine compound severally in different solvents and mixing the resultant solutions. The solvents which are usable for the solution or dispersion of the binder resin and the photoelectroconductive phthalocyanine compound are organic solvents including aromatic hydrocarbons such as benzene and toluene, cyclic ethers such as tetrahydrofuran and dioxane, halogen-containing hydrocarbons such as chloroform, dichloromethane, and dichloroethane, ketones such as acetone and methylethyl ketone, esters such as ethyl acetate, and cellosolves such as methyl cellosolve, for example.

In the preparation of the coating liquid mentioned above, the photoelectroconductive phthalocyanine compound in a ratio in the range of 3 to 50% by weight, preferably 5 to 30% by weight, based on the amount of the binder resin.

The concentrations of the photoelectroconductive phthalocyanine compound and the binder resin dissolved or dispersed in their solvents are both desired to be generally in the range of 0.5 to 50% by weight, preferably 5 to 30% by weight.

The thickness of the photosensitive layer is in the range of 2 to 10 µm, preferably 3 to 6 µm. If the wall thickness is larger than the upper limit of the range, there arises a disadvantage that the etching treatment tends to give rise to side edges and consequently tends to scrape off fine lines. If the wall thickness is smaller than the lower limit of the range, there ensues a disadvantage that the photosensitive layer suffers from inferior chargeability.

The coating liquid prepared for the formation of the photosensitive layer of the type to be used as positively charged may, for the purpose of further improving the electrophotographic properties thereof, incorporate additionally therein as a sensitiger at least one compound selected from among organic compounds of polybasic acids such as, for example, compounds represented by the following general formulas III, IV, and V and succinic anhydride and maleic anhydride. wherein X¹ to X⁵ are equally or unequally each for hydrogen atom, fluorine atom, -COOH group, or a -NO₂ group), wherein Y¹ and Y⁴ in are equally or unequally each for hydrogen atom, fluorine atom, -COOH group, or -NO₂ group, and wherein Z¹ and Z are equally or unequally each for hydrogen atom, fluorine atom, -COOH group, or -NO₂ group.

Typical examples of the sensitiser include succinic anhydride, maleic anhydride, phthalic acid, tetrafluorophthalic acid, 4-nitrophthalic acid, phthalic anhydride, tetrafluorophthalic anhydride, 4-nitorphthalic anhydride, trimellitic acid, trimellitic anhydride, benzoic acid, pentafluorobenzoic acid, and tetrafluorobenzoic acid. Among other sensitive enhancers mentioned above, succinic anhydride, tetrafluorophthalic anhydride, benzoic acid, pentafluorobenzoic acid, and tetrafluorobenzoic acid prove to be preferable and tetrafluorophthalic anhydride, pentafluorobenzoic acid, and tetrafluorobenzoic acid prove to be particularly preferable.

The sensitiger is preferable to be used in a ratio in the range of 0.01 to 10% by weight, preferably below 2.0% by weight, based on the amount of the photoelectroconductive phthalocyanine compound.

The coating liquid prepared for the formation of the photosensitive layer which is to be used as charged to negative polarity may, for the purpose of further improving the electrophotographic properties thereof, incorporate additionally therein an electric charge transferring substance such as, for example, an oxazole derivative, an oxadiazole derivative, a pyrazoline derivative, a hydrazone derivative, or a triphenylamine derivative and/or an aminotriazine resin.

It is preferable to use a hydrazone derivative represented by the following general formula VI as an electric charge transferring substance. wherein R¹ and R are each an aryl group or an aralkyl group and R³ is hydrogen atom, an alkyl group of 1 to 4 carbon atoms, a benzyl group, an alkoxy group of 1 to 4 carbon atoms, a phenoxy group, or a benzyloxy group.

As typical examples of the hydrazine compounds represented by the aforementioned general formula, the following compounds may be cited.

The aminotriazone resins which are usable herein include melamine resin, benzoguanamine resin, acetoguanamine resin, CTU-guanamine resin (proprietary product of Ajinomoto Co., Inc.), and cyclohexyl guanamine, for example. It is particularly preferable to use cyclohexyl carboguanamine resin among other aminotriazine resins mentioned above.

The aminotriazine resin is an aminotriazine resin composition, namely the oxymethylated or alkyloxymethylated product of aminotriazine, obtained by the reaction of aminotriazine with formaldehyde optionally further with an alcohol such as butanol. It is used either in the unmodified form thereof or in a form suitably condensed by dehydration. It is preferable to use the aforementioned electric charge transferring substance and/or aminotriazine resin in a ratio not exceeding 60% by weight, preferably falling in the range of 0.1 to 20% by weight.

The electroconductive substrate to be used in the present invention is not particularly limited. The electroconductive substrates which are usable effectively herein include monometallic plates such as aluminum plate and zinc plate, bimetal plates such as copper-aluminum plate, copper-stainless steel plate, and chromium-copper plate, and trimetallic plates such as chromium-copper-aluminum plate, chromium-copper iron plate, and chromium-copper-aluminum plate invariably possessing a hydrophilic surface and finding popular use. The thickness of the electroconductive substrate is desired to be approximately in the range of 0.05 to 0.5 mm.

Particularly, in the case of a substrate having an aluminum surface, it is preferable to have undergone a surface treatment such as abrasion with sand, immersion in an aqueous solution of sodium silicate or potassium fluorozirconate, or anodix oxidation.

The treatment of anodic oxidation can be carried out by placing an aluminum plate in an electrolytic solution formed of the solution of an inorganic acid such as phosphoric acid, chromic acid, sulfuric acid, or boric acid, an organic acid such as oxalic acid or sulfamic acid, or any of the salts of such acids, and flowing an electric current through the aqueous solution with the aluminum plate as an anode. Further, it is preferable to provide an intermediate layer comprising a resin having a composition within the range of the present invention having higher acid value than the binder resin in the sensitive layer between the electroconductive substrate and electrophotosensitive layer in order to enhance the printing quality in the present invention.

The electrophotographic plate-making quality matric plate of the present invention is not discriminated on account of the method to be employed for the production thereof. This production can be accomplished by any of the methods heretofore known to the art. In accordance with the conventional electrophotographic technique, for example, a toner image is obtained on a photosensitive layer by first uniformly charging the photosensitive layer in a dark place with a corona charging device, subjecting the charged photosensitive layer to the reflection image exposure using such a light source as a tungsten lamp, a halogen lamp, a xenon lamp, or a fluoroescent lamp, the tight-contact image exposure through a transparent positive film, or the scanning exposure with a laser beam such as a He-Ne laser, an argon laser, or a semiconductor laser thereby forming an electrostatic latent image therein, developing this latent image with a toner, and thermally fixing the developed toner image.

The toner must be hydrophobic and capable of receiving ink, adhesive to the matric plate so much as to withstand the impact of printing, and resistant to the action of an alkaline aqueous etching liquid to be used during the course of etching. As the electrophotographic developer, since a liquid developer excels a powdery developer in resolving power, it is more preferable to use the former developer than the latter developer. For the toner to fulfill the requirements mentioned above, the resin which the toner is preferable to contain is styrene resin, acrylic resin, styrene-acrylic resin, styrene-methacrylic resin, polyester resin, or epoxy resin, for example. The dispersant for the toner is an organic solvent possessing a low dielectric constant and a high insulating capacity. An isoparaffin type hydrocarbon, for example, is used preferable. The toner may incorporate therein a pigment or dye for the purpose of coloration or an electric charge regulating agent for the purpose of imparting positive charge or negative charge in an amount incapable of exerting any adverse effect upon the stability and the fixing property of the toner and yet fit for the purpose for which the toner is used.

When the plate-making matrix plate on which the toner image has been formed as described above is immersed in an alkaline dissolving liquid, the photosensitive layer in the non-image part not masked with the toner image is dissolved and removed to expose the hydrophilic surface of the electroconductive substrate and the image part of the toner image is allowed to remain on the surface of the substrate to give rise to a lithographic printing plate aimed at.

The alkaline dissolving liquids which are effectively usable for the solution and removal of the photosensitive layer in the non-image part include alkaline aqueous solution and removal of the photosensitive layer in the non-image part include alkaline aqueous solutions of inorganic salts such as sodium silicate, sodium phosphate, sodium hydroxide, and sodium carbonate, alkaline aqueous solutions of organic amines such as triethanol amine and ethylene diamine, and solutions incorporating therein organic solvents such as ethanol, benzyl alcohol, ethylene glycol, and glycerol or surfactants, for example. An alkaline aqueous etching liquid of the following composition, for example, can be used advantageously.

| | |
|---|---|
| Edta-4H | 4 g |
| Benzyl alcohol | 30 g |
| Monoethanol amine | 5 g |
| Triethanol amine | 60 g |
| NaOH | 25 g |

Water added to dilute the compounds mentioned above to a total volume of 1 liter.

The electrophotographic plate-making quality matric plate may be otherwise used as a laser printer (OPC) quality electrophotographic sensitive material. In the laser printer, the developed toner is transferred onto a sheet of paper and fixed thereon.

Now, the present invention will be described more specifically below with reference to production examples and working examples. Wherever "parts" and "percentages" are mentioned, they are meant as "parts by weight" and "percents by weight" unless otherwise specified.

### Production Example 1 [Production of F₈(PhS)₈ZnPc]

### (1) Synthesis of starting material

In a four-neck flask having an inner volume of 200 ml, 19.6 g (98 m.mols ) of 3,4,5,6-tetrafluiorophthalonitrile, 21.6 g (196 m.mols) of thiophenol, 17.1 g (294 m.mols) of potassium fluoride (KF), and 100 ml of acetonitrile were placed and stirred at 50°C for reaction for 12 hours. Then, the reaction mixture was cooled to room temperature. The yellow solid which formed consequently in the mixture was separated by filtration. The cake thus obtained was purified by washing first with methanol and then with hot water, to obtain 34.5 g of 3,6-difluoro-4,5-bisphenylthiophthalonitrile (yield: 92.5 mol% based on 3,4,5,6-tetrafluoronitrile).

### (2) Synthesis of F₈(PhS)₈ZnPc

In a four-neck flask having an inner volume of 100 ml, 10 g (26.2 m.mols) of 3,6-difluoro-4,5-bisphenyl thiophthalonitrile, 3.14 g (9.8 m.mols) of zinc iodide, and 50 ml of benzonitrile were placed and then stirred at 175°C for reaction for 6 hours. Then, the reaction mixture was cooled. The green solid consequently formed in the reaction mixture was separated by filtration, washed in a Soxhlet extractor with methanol, benzene, and acetone sequentially in the roder mentioned, to obtain F₈(PhS)₈ZnPc in a yield of 79.4 mol % based on 3,6-difluoro-4,5-bisphenylthiophthalonitrile.

### Production Example 2 [Production of copolymer]

The copolymer can be produced as follows, for example. In a separable flask provided with a stirrer, a thermometer, a condenser, a nitrogen inlet tube, a monomer mixture dropping funnel, and a polymerization initiator dropping funnel, 40 parts of isopropanol is placed as a solvent and then nitrogen is introduced through the nitrogen inlet tube to displace the air entrapped in the flask with the nitrogen. Subsequently, 60 parts of a monomer mixture is placed in the monomer mixture dropping funnel and 0.1 part of azobisisobutyronitrile is placed in the polymerization initiator dropping funnel. With the inner temperature of the flask kept at 80°C, the monomer mixture and the polymerization initiator are dropped into the flask over a period of two hours. The mixture in the flask is heated at 80°C for two hours and then at 85° to 95°C for two hours and then cooled.

### Example 1

In a paint shaker dispersion device, 1.5 parts of F₈(o-MePhS)₈ZnPc, 0.05 part of pentafluorobenzoic acid, 12.0 parts of a copolymer obtained from the monomer mixture (P-1), and 83 parts of dichloroethane were shaken for dispersion for 2 hours. The resultant dispersion was applied on an aluminum plate which had been abraded in a thickness of 0.15 mm with a barcoater and further treated for anodic oxidation. The applied layer of the dispersant was dried with hot wind at 60°C for 30 minutes and then desiccated under a vacuum (1 mmHg) at 100°C for 2 hours, to form a photosensitive layer. The film (photosensitive layer) thus obtained had a thickness of 5 µm.

The monolayer type electrophotographic sensitive material obtained as an electrophotographic plate-making quality matric plate as described above was positively charged at +6.0 kV with an electrostatic paper analyzer (produced by Kawaguchi Denki K.K. and marketed under product code of "SP-428").

The photosensitive material was then retained in a dark place for 5 seconds, exposed to white light (from a tungsten lamp) with an illuminance of 5 luxes for 5 seconds to test for charging properties [surface potential (V₀), potential (V₅) after 5 seconds retention in the dark place, and amount of exposure required for the potential existing before the exposure to attenuate to 1/2 by exposure (E_{1/2}) (Lux.sec)]. It was then exposed to a monochromatic light of 780 nm separated by dispersion with a spectral filter to 0.5 µw/cm to determine half-value exposure energy sensitivity (µJ/cm).

Then, the monolayer type electrophotographic sensitive material was immersed in an aqueous 0.5% sodium hydroxide solution and then washed with water to remove the photosensitive layer. In this case, the alkali dissolving property was evaluated in terms of the speed of removal of the photosensitive layer.

Subsequently, the same monolayer type electrophotographic sensitive material separately formed on an abraded aluminum plate was subjected to platemaking by the liquid developing process using a TTP laser plate-making device produced by Toppan Printing Co., Ltd. Corona charging was effected at +6 kV. The electrostatic latent image was developed with a negatively polarized developer. The developed image was thermally fixed to form a toner image.

The toner image thus formed was washed out with an alkaline aqueous etching solution and washed with water to produce a lithographic printing plate.

The printing plate thus produced was set in place in an offset printing device and used to produce prints by the conventional process. The initially produced prints and the prints produced after 100,000th print were evaluated for degree of scumming and clarity of print.

The results of the evaluation of electrophotographic properties, alkali dissolving property, and printing quality are shown in Table 2.

### Examples 2 to 17

Electrophotographic plate-making quality matric plates were produced by following the procedure of Example 1, except that varying photoelectroconductive phthalocyanine compounds indicated in Table 1, copolymers obtained from various monomer mixtures (P-1) to (P-8), and sensitigers were used in the place of F₈(o-MePhS)₈ZnPc and the copolymer of the monomer mixture (P-1). They were evaluated for electrophotographic properties, alkali-dissolving property, and printing quality. The results are shown in Table 2. The electrophotographic sensitive materials produced as described above were left standing in a room illuminated with a fluorescent lamp for 2 months and then tested for electrophotographic properties and printing quality. The properties showed virtually no difference before and after the two months' standing.

### Controls 1 to 6

Electrophotographic plate-making quality matric plates were produced by following the procedure of Example 1, except that various photoelectroconductive phthalocyanine compounds indicated in Fig. 1, the copolymers obtained from the monomer mixtures of (P-1) and (P-8) and the monomer mixtures, (S-1) to (S-5), shown below produced in the same manner as in Production Example 2, and sensitigers. They were similarly evaluated for electrophotographic properties, alkali-dissolving property, and printing quality. The results are shown in Table 2.
(S-1) Acrylic acid/butyl acrylate/butyl methacrylate (25/20/55),
(S-2) Methacrylic acid/styrene/isopropyl acrylate (30/15/55),
(S-3) Methacrylic acid/methyl acrylate/ethyl methacrylate (15/60/25),
(S-4) Acrylic acid/styrene/ethyl acrylate/methyl methacrylate (25/8/20/47), and
(S-5) Acrylic acid/butyl acrylate/methyl methacrylate/2-hydroxyethyl methacrylate (10/40/40/10)
Surface potential, V₀ (V) Potential in dark place, V₅ (V)
Half-value exposure amount (E_{1/2})
Exposed to tungsten lamp (Lux·sec)
Exposure to light of 780 nm (µJ/cm)
Speed of alkali dissolution (sec) Printing quality
A: Capable of producing 100,000 very clear prints free from smeared background and from worn lines.
B: Capable of producing 100,000 clear prints free from smeared background and not from worn lines.
C: Productive of prints suffering from smeared background or inferior clarity.
D: Peeling of plate surface observed after production of 100,000 prints.
E: No toner image obtained and no printing attained.

### Examples 18 to 27

Electrophotographic plate-making quality matric plates were produced by following the procedure of Example 1, except that the various photoelectroconductive phthalocyanine compounds indicated in Table 3 and the copolymers obtained from the monomer mixtures of (P-1) to (P-8) were used in the place of the F₈(o-MePhS)₈ZnPc and the copolymer of the monomer mixture of (P-1). The monolayer type electrophotographic sensitive materials obtained as the electrophotographic plate-making quality matric plates as described above were negatively charged at -6.0 kV with an elecrtrostatic paper analyzer. They were evaluated for electrophotographic properties, alkali-dissolving property, and printing quality in the same manner as in Example 1. The results are shown in Table 4.

## Claims

1. An electrophotographic matrix plate comprising an electroconductive substrate having a photosensitive layer comprising an alkali-soluble binder resin and a photoconductive fluorinated zinc phthalocyanine compound, characterised in that the photoconductive compound is an octafluoro zinc phthalocyanine represented by the general formula I: wherein R is a -SZ group, where Z is a phenyl group, a phenyl group substituted with an alkyl group of 1 to 5 carbon atoms, or a naphthyl group; and in that the binder resin is a copolymer obtainable by polymerising a monomer mixture comprising (a) one or more hydroxyalkyl acrylate(s) and/or hydroxyalkyl methacrylate(s), (b) at least one copolymerisable unsaturated carboxylic acid, (c) at least one styrene compound, and (d) at least one acrylic ester other than the hydroxyalkyl acrylate(s) of (a), and optionally (e) at least one methacrylic ester other than the hydroxyalkyl methacrylate(s) of (a).

2. A matrix plate as claimed in Claim 1, characterised in that the binder resin is a copolymer of a number average molecular weight in the range of 1,000 to 50,000 obtainable by the polymerisation of a monomer mixture composed of (a) 0.5 to 40% by weight of one or more hydroxyalkyl acrylate(s) and hydroxyalkyl methacrylate(s) having alkyl groups of 2 to 10 carbon atoms, (b) 10 to 40% by weight of at least one copolymerisable carboxylic acid selected from acrylic acid, methacrylic acid, and itaconic acid, (c) 10 to 70% by weight of at least one styrene compound, (d) 5 to 50% by weight of at least one acrylic ester selected from alkyl acrylates having alkyl groups of 1 to 12 carbon atoms and cycloalkyl acrylates having cycloalkyl groups of 5 to 7 carbon atoms, and optionally (e) up to 40% by weight of at least one methacrylic ester selected from the group consisting of alkyl methacrylates having alkyl groups of 1 to 12 carbon atoms and cycloalkyl methacrylates having cycloalkyl groups of 5 to 7 carbon atoms.

3. A matrix plate as claimed in Claim 1 or 2, characterised in that the photosensitive layer, when it is to be charged to positive polarity in use, contains a sensitizer.

4. A matrix plate as claimed in Claim 3, characterized in that the sensitizer is at least one compound selected from compounds represented by the following general formulas, III, IV, and V, succinic anhydride, and maleic anhydride: wherein X¹ to X⁵ are, either equally or non-equally, a hydrogen atom, fluorine atom, -COOH group, or -NO₂ group, wherein Y¹ to Y⁴ are, either equally or non-equally, a hydrogen atom, fluorine atom, -COOH group, or -NO₂ group, and wherein Z¹ and Z are, either equally or non-equally, a hydrogen atom, fluorine atom, -COOH group, or -NO₂ group.

5. A matrix plate as claimed in Claim 1 or 2, characterised in that the photosensitive layer, when it is to be charged to negative polarity in use, contains at least one charge transferring substance selected from oxazole derivatives, oxadiazole derivatives, pyrazoline derivatives, hydrazone derivatives, and triphenylamine derivatives.

6. A matrix plate as claimed in Claim 5, characterized in that the charge transferring substance is represented by the following general formula VI: wherein R¹ and R are each an aryl group or an aralkyl group and R³ is hydrogen atom, an alkyl group of 1 to 4 carbon atoms, a benzyl group, an alkoxy group of 1 to 4 carbon atoms, a phenoxy group, or a benzyloxy group.

7. A matrix plate as claimed in Claim 1 or 2, characterised in that the photosensitive layer, when it is to be charged to negative polarity in use, contains an aminotriazine resin.

8. A matrix plate as claimed in Claim 7, characterised in that the aminotriazine resin is at least one composition selected from benzoguanamine resin compositions, cyclohexylcarboguanamine resin compositions, melamine resin compositions, and acetoguanamine resin compositions.

9. A matrix plate as claimed in Claim 7, characterized in that the aminotriazine resin and a composition thereof are respectively the condensate of oxymethylated aminotriazine and the condensate of alkylether oxymethylated aminotriazine.

10. A lithographic printing plate obtainable by forming a toner image by the electrophotographic process on an electrophotographic matrix plate as claimed in any of Claims 1 to 9, fixing the toner image, and then removing the non-image part of the toner image with an alkaline etching liquid.

## Patentansprüche

1. Elektrofotografische Matrixplatte, die ein elektrisch leitfähiges Substrat enthält, das eine fotoempfindliche Schicht besitzt, die ein alkalilösliches Binderharz und eine fotoleitfähige, fluorierte Zink-Phthalocyanin-Verbindung aufweist, dadurch gekennzeichnet, daß die fotoleitfähige Verbindung ein Octafluor-Zink-Phthalocyanin ist, dargestellt durch die allgemeine Formel I: wobei R eine -SZ-Gruppe ist, in der Z eine Phenylgruppe, eine Phenylgruppe, die mit einer Alkylgruppe mit 1 bis 5 Kohlenstoffatomen substituiert ist, oder eine Naphthylgruppe ist, und daß das Binderharz ein Copolymer ist, das durch Polymerisieren einer Monomermischung erhältlich ist, die (a) ein oder mehrere Hydroxyalkyl-acrylat(e) und/oder Hydroxyalkyl-methacrylat(e), (b) mindestens eine copolymerisierbare, ungesättigte Carbonsäure, (c) mindestens eine Styryl-Verbindung und (d) mindestens einen Acrylsäureester aufweist, der sich von dem (den) Hydroxyalkyl-acrylat(en) unter (a) unterscheidet, sowie wahlweise (e) mindestens einen Methacrylsäureester, der sich von dem (den) Hydroxyalkyl-methacrylat(en) aus (a) unterscheidet.

2. Matrixplatte gemäß Anspruch 1, dadurch gekennzeichnet, daß das Binderharz ein Copolymer mit einem zahlenmittleren Molekulargewicht im Bereich von 1000 bis 50000 ist, das durch Polymerisieren einer Monomermischung erhältlich ist, die zusammengesetzt ist aus (a) 0,5 bis 40 Gew.-% von einem oder mehr Hydroxyalkyl-acrylat(en) und Hydroxyalkyl-methacrylat(en) mit Alkylgruppen von 2 bis 10 Kohlenstoffatomen, (b) 10 bis 40 Gew.-% mindestens einer copolymerisierbaren Carbonsäure, ausgewählt aus Acrylsäure, Methacrylsäure und Itaconsäure, (c) 10 bis 70 Gew.-% mindestens einer Styryl-Verbindung, (d) 5 bis 50 Gew.-% von mindestens einem Acrylsäureester, ausgewählt aus Alkyl-acrylaten mit Alkylgruppen von 1 bis 12 Kohlenstoffatomen und Cycloalkyl-acrylaten mit Cycloalkylgruppen von 5 bis 7 Kohlenstoffatomen und wahlweise (e) bis zu 40 Gew.-% von mindestens einem Methacrylsäureester, der aus der Gruppe gewählt ist, die aus Alkyl-methacrylaten mit Alkylgruppen von 1 bis 12 Kohlenstoffatomen und Cycloalkyl-methacrylaten mit Cycloalkylgruppen von 5 bis 7 Kohlenstoffatomen besteht.

3. Matrixplatte gemäß Anspruch 1 oder 2, dadurch gekennzeichnet, daß die fotoempfindliche Schicht, wenn sie auf positive Polarität im Einsatz aufgeladen werden soll, einen Sensibilisator enthält.

4. Matrixplatte gemäß Anspruch 3, dadurch gekennzeichnet, daß der Sensibilisator mindestens eine Verbindung ist, die aus den Verbindungen, die durch die folgenden allgemeinen Formeln III, IV und V repräsentiert werden, sowie aus Bernsteinsäureanhydrid und Maleinsäureanhydrid ausgewählt ist: wobei X¹ bis X⁵ entweder gleich oder ungleich sind und ein Wasserstoffatom, ein Fluoratom, eine -COOH-Gruppe oder eine -NO₂-Gruppe darstellen, wobei Y¹ bis Y⁴ entweder gleich oder ungleich sind und ein Wasserstoffatom, ein Fluoratom, eine -COOH-Gruppe oder eine -NO₂-Gruppe darstellen, und wobei Z¹ und Z entweder gleich oder ungleich sind und ein Wasserstoffatom, ein Fluoratom, eine -COOH-Gruppe oder eine -NO₂-Gruppe darstellen.

5. Matrixplatte gemäß Anspruch 1 oder 2, dadurch gekennzeichnet, daß die fotoempfindliche Schicht, wenn sie auf negative Polarität im Einsatz aufgeladen werden soll, mindestens eine Ladungsübertragungs-Substanz enthält, die aus Oxazol-Derivaten, Oxadiazol-Derivaten, Pyrazolin-Derivaten, Hydrazon-Derivaten und Triphenylamin-Derivaten ausgewählt ist.

6. Matrixplatte gemäß Anspruch 5, dadurch gekennzeichnet, daß die Ladungsübertragungs-Substanz durch die folgende allgemeine Formel VI dargestellt wird: wobei R¹ und R jeweils eine Aryl-Gruppe oder eine Aralkyl-Gruppe ist und R³ ein Wasserstoffatom, eine Alkylgruppe mit 1 bis 4 Kohlenstoffatomen, eine Benzyl-Gruppe, eine Alkoxy-Gruppe mit 1 bis 4 Kohlenstoffatomen, eine Phenoxy-Gruppe oder eine Benzyloxy-Gruppe ist.

7. Matrixplatte gemäß Anspruch 1 oder 2, dadurch gekennzeichnet, daß die fotoempfindliche Schicht, wenn sie auf eine negative Polarität im Einsatz aufgeladen werden soll, ein Aminotriazin-Harz enthält.

8. Matrixplatte gemäß Anspruch 7, dadurch gekennzeichnet, daß das Aminotriazin-Harz mindestens eine Zusammensetzung aufweist, die aus Benzoguanamin-Harz-Zusammensetzungen, Cyclohexylcarboguanamin-Harz-Zusammensetzungen, Melamin-Harz-Zusammensetzungen und Acetoguanamin-Harz-Zusammensetzungen ausgewählt ist.

9. Matrixplatte gemäß Anspruch 7, dadurch gekennzeichnet, daß das Aminotriazin-Harz bzw. eine Zusammensetzung davon das Kondensat aus oxymethyliertem Aminotriazin oder das Kondensat aus Alkyletheroxymethyliertem Aminotriazin ist.

10. Lithografische Druckplatte, die dadurch erhältlich ist, daß durch den elektrofotografischen Prozeß auf einer elektrofotografischen Matrixplatte gemäß einem der Ansprüche 1 bis 9 ein Toner-Bild gebildet wird, das Toner-Bild fixiert und dann der nichtbildgebende Teil des Toner-Bildes mit einer alkalischen Ätzflüssigkeit entfernt wird.

## Revendications

1. Plaque matricielle électrophotographique comprenant un substrat électroconducteur ayant une couche photosensible comprenant une résine liante soluble en milieu alcalin et un composé zinc-phtalocyanine fluorée photoconducteur, caractérisée en ce que le composé photoconducteur est une zinc-octafluorophtalocyanine représentée par la formule générale I : dans laquelle R est un radical -SZ, où Z est un radical phényle, un radical phényle substitué par un radical alcoyle de 1 à 5 atomes de carbone, ou un radical naphtyle; et en ce que la résine liante est un copolymère pouvant être obtenu par polymérisation d'un mélange de monomères comprenant :
(a) un ou plusieurs acrylates d'hydroxyalcoyle et/ou méthacrylates d'hydroxyalcoyle;
(b) au moins un acide carboxylique insaturé copolymérisable;
(c) au moins un composé styrénique, et
(d) au moins un ester acrylique autre que le ou les acrylates d'hydroxyalcoyle de (a), et facultativement,
(e) au moins un ester méthacrylique autre que le ou les méthacrylates d'hydroxyalcoyle de (a).

2. Plaque matricielle suivant la revendication 1, caractérisée en ce que la résine liante est un copolymère d'un poids moléculaire moyen en nombre situé dans l'intervalle de 1000 à 50 000, pouvant être obtenu par la polymérisation d'un mélange de monomères composé de :
(a) 0,5 à 40% en poids d'un ou de plusieurs acrylates d'hydroxyalcoyle et méthacrylates d'hydroxyalcoyle ayant des radicaux alcoyle de 2 à 10 atomes de carbone;
(b) 10 à 40% en poids d'au moins un acide carboxylique copolymérisable, choisi parmi l'acide acrylique, l'acide méthacrylique et l'acide itaconique;
(c) 10 à 70% en poids d'au moins un composé styrénique;
(d) 5 à 50% en poids d'au moins un ester acrylique choisi parmi les acrylates d'alcoyle ayant des radicaux alcoyle de 1 à 12 atomes de carbone et les acrylates de cycloalcoyle ayant des radicaux cycloalcoyle de 5 à 7 atomes de carbone, et facultativement,
(e) jusqu'à 40% en poids d'au moins un ester méthacrylique choisi parmi le groupe consistant en les méthacrylates d'alcoyle ayant des radicaux alcoyle de 1 à 12 atomes de carbone et les méthacrylates de cycloalcoyle ayant des radicaux cycloalcoyle de 5 à 7 atomes de carbone.

3. Plaque matricielle suivant la revendication 1 ou 2, caractérisée en ce que la couche photosensible, lorsqu'elle doit être chargée en polarité positive lors de l'utilisation, contient un sensibilisateur.

4. Plaque matricielle suivant la revendication 3, caractérisée en ce que le sensibilisateur est au moins un composé choisi parmi les composés représentés par les formules générales (III), (IV) et (V) suivantes, l'anhydride succinique et l'anhydride maléique : dans laquelle X¹ à X⁵ sont, identiquement ou non, un atome d'hydrogène, un atome de fluor, un radical -COOH ou un radical -NO₂; dans laquelle Y¹ à Y⁴ sont, identiquement ou non, un atome d'hydrogène, un atome de fluor, un radical -COOH ou un radical -NO₂, et dans laquelle Z¹ et Z sont, identiquement ou non, un atome d'hydrogène, un atome de fluor, un radical -COOH ou un radical -NO₂.

5. Plaque matricielle suivant la revendication 1 ou 2, caractérisée en ce que la couche photosensible, lorsqu'elle doit être chargée en polarité négative lors de l'utilisation, contient au moins une substance de transfert de charge choisie parmi les dérivés de l'oxazole, les dérivés de l'oxadiazole, les dérivés de la pyrazoline, les dérivés de l'hydrazone et les dérivés de la triphénylamine.

6. Plaque matricielle suivant la revendication 5, caractérisée en ce que la substance de transfert de charge est représentée par la formule générale (VI) suivante : dans laquelle R¹ et R sont chacun un radical aryle ou un radical aralcoyle et R³ est un atome d'hydrogène, un radical alcoyle de 1 à 4 atomes de carbone, un radical benzyle, un radical alcoxy de 1 à 4 atomes de carbone, un radical phénoxy ou un radical benzyloxy.

7. Plaque matricielle suivant la revendication 1 ou 2, caractérisée en ce que la couche photosensible, lorsqu'elle doit être chargée en polarité négative lors de l'utilisation, contient une résine de type aminotriazine.

8. Plaque matricielle suivant la revendication 7, caractérisée en ce que la résine de type aminotriazine est au moins une composition choisie parmi les compositions résiniques de benzoguanamine, les compositions résiniques de cyclohexylcarboguanamine, les compositions résiniques de mélamine et les compositions résiniques d'acétoguanamine.

9. Plaque matricielle suivant la revendication 7, caractérisée en ce que la résine de type aminotriazine et une composition de celle-ci sont, respectivement, le condensat d'aminotriazine oxyméthylée et le condensat d'un alcoyléther d'aminotriazine oxyméthylée.

10. Plaque d'impression lithographique pouvant être obtenue en formant une image de toner par le procédé électrophotographique sur une plaque matricielle électrophotographique suivant l'une quelconque des revendications 1 à 9, en fixant l'image de toner et ensuite, en éliminant la partie non-image de l'image de toner au moyen d'un liquide alcalin de gravure.
